

J. M. GERARD.

PROCESS FOR THE MANUFACTURE OF CARBON BLACK AND LAMPBLACK.  
APPLICATION FILED OCT. 8, 1917.

1,278,137.

Patented Sept. 10, 1918.



# UNITED STATES PATENT OFFICE.

JULIAN M. GERARD, OF NEW YORK, N. Y.

## PROCESS FOR THE MANUFACTURE OF CARBON-BLACK AND LAMPBLACK.

1,278,137.

Specification of Letters Patent. Patented Sept. 10, 1918.

Application filed October 8, 1917. Serial No. 195,299.

To all whom it may concern:

Be it known that I, JULIAN M. GERARD, citizen of the United States, residing at New York, in the county of New York and State of New York, have invented certain new and useful Improvements in Processes for the Manufacture of Carbon-Black and Lampblack, of which the following is a specification.

10 My invention relates to a new and improved method for the manufacture of lampblack.

Lampblack, as heretofore manufactured, has been chiefly made by burning natural gas, various oils, and the like, in such a manner that part of the carbon therein is consumed and the remainder is present in the gases of combustion, and collecting this unconsumed carbon usually by causing the flame to impinge upon a cooled surface. Such processes are extremely wasteful, because a large amount of the carbon is consumed in producing the heat of the flame, and a considerable amount of the unconsumed carbon cannot be collected upon the cooled surface.

According to my invention, the particles of carbon remaining after the incomplete combustion of the substances consumed, are collected by means of electrical precipitation when the gas is cooled to a suitable temperature, to be later disclosed herein, and the carbon is removed from the collecting surfaces without scraping or other mechanical movements of one particle with respect to the others. Because of the fact that the particles are removed from a current of the cooled gas, they collect in an extremely fine state of subdivision, so much so, that no mechanical means such as scrapers or the like, can be used or are necessary. In fact, experience has shown that the vibration of the air, due to a loud sound, is sufficient to dislodge the carbon particles from their collecting surfaces. As a result of this, and because the particles are dislodged without the use of scrapers or similar means which would tend to move the carbon particles with respect to each other and compact them, a quality of lampblack is obtained of a much finer quality than that heretofore secured from the old methods above mentioned.

I have also found it desirable and possible to divide the unconsumed carbon particles

in the flame into two grades or qualities by 55 allowing the flame to first impinge upon a cool surface as in the old method, and then collecting the remaining particles by means of electrical precipitation. By this method an especially fine quality of lampblack is 60 secured in the precipitator.

This fine grade secured in the electrical precipitator is easily miscible with water when the lampblack is made from natural gas to which my invention is particularly 65 directed, and has an unusual brilliancy and coloring power. My invention is not limited to natural gas as the source for the lampblack, but it may also be extended to other sources thereof, such as oils or the like. 70

Further objects of my invention will be set forth in the following description and drawings, which illustrate a mechanism that may be used for carrying out my invention.

Figure 1 is a diagrammatic cross-section 75 along line 1—1 of Fig. 2.

Fig. 2 is a longitudinal cross-section shown diagrammatically.

Fig. 3 is a plan view.

The natural gas is led into the building 1, 80 into the burners 16, mounted upon the supports 15. The ventilation of the building is so controlled that instead of the proportion of air now supplied, sufficient air is supplied to the natural gas of the kind 85 found in the Southern part of the United States, so as to cause it to produce between 2 and 3 pounds of lampblack per thousand cubic feet. As practically all of the lampblack particles in the fluid are collected by 90 the method of precipitation herein shown, I have found it expedient in practice to cause the burning of the hydrocarbon gases to be effected with the minimum amount of oxygen necessary to maintain combustion. The burners cause the flames which are full of unconsumed particles of carbon, to impinge upon the cylinders 10, which are suitably cooled by air or water in the manner well known to the art. The deposit 100 formed upon these cylinders 10 is scraped off by the scrapers 11, which causes the lampblack to fall into the pipes 12, from which it is removed by means of the screw conveyors 20 operating in the chambers 13, 105 to be discharged into the packing house 5, from the mouths of the chambers 13.

In this manner a certain amount of the

carbon is deposited upon the cool cylinders 10, and this amount is preferably about one pound for every thousand cubic feet.

The remaining gas and particles are led 5 into pipe 2 and then drawn through it by any suitable means, so arranged, as not to disturb the ventilation of the building 1 as before mentioned. A fan 3, if desired, may be employed to cause an artificial draft.

10 In this pipe 2 the flames are cooled to about 400 degrees C. at which temperature the ionic discharge caused by the electrical precipitator causes the collection of the carbon particles in a very loose and finely divided condition, and are thence sent through the tubes 6, in which the conductors 7 comprising smooth, uninsulated wires, are placed along their axes. The tubes are provided in a suitable number, so as not to supply 15 any wire 7 with too much gas or particles.

15 The wires 7, which are the active conductors, are furnished with a unidirectional current of from fifty thousand to seventy-five thousand volts, by electrical apparatus of a suitable kind, as this voltage has been found 20 suitable for precipitating the lampblack in the finely divided form before mentioned.

25 As here illustrated, a current from a suitable generator 34 is sent into a transformer 30 22, comprising a primary coil 24 and a secondary coil 23, so that the current has its voltage raised to the required amount.

30 The current is then sent through a rectifier 25 of any suitable kind, and is supplied 35 therefrom to the wire 7. The current supplied to the wire 7 may be altered, if desired. Resistances 29 and 32, and capacities 28 and 33, self-inductances 30 and 31 and 40 spark gaps 26 and 27 are arranged in the secondary circuit, so that the oscillation of the proper frequency and suitable damping factors are produced. The corona or brush 45 discharge is produced, a disruptive discharge being avoided. If the carbon deposit becomes 50 too heavy, so that there is danger of a disruptive discharge, then some of the deposit is removed while the electrical precipitation is temporarily stopped.

55 Under ordinary circumstances, gravity or a slight vibration removes the deposit with sufficient rapidity to prevent a disruptive discharge. If a disruptive discharge is caused by the collection of the particles upon the wires 7, the polarity thereof is temporarily reversed, which causes the clearing of the wire 7 of the accumulation thereon. Even if a disruptive discharge does take place, it has little or no effect upon the extreme fineness of the deposits.

60 The building 5, which constitutes the packing house, is connected to the ground so that the tubes are also so connected, and serve as collectors. The cylinders 10 are made of nickel, zinc, or copper, or some other non-oxidizing material. A sheet of gauze 17 may

be interposed between the flames and the cylinders 10, to cool the flames. Instead of the specific means for producing a high tension current for the brush or corona discharge above mentioned, any well-known 70 means may be employed, and an alternating current may be used.

I claim:

1. A method of producing lampblack which consists in electrically precipitating 75 the unoxidized carbon particles suspended in the gaseous products resulting from the incomplete oxidation of a hydrocarbon, the voltage employed in said precipitation being such that the said unoxidized carbon is collected in a finely divided form.

2. A method of producing lampblack which consists in electrically precipitating unoxidized carbon particles suspended in the gaseous products resulting from the incomplete oxidation of a hydrocarbon, the temperature of said carbon particles suspended in the gaseous products being less than the temperature at which the said oxidation took place, the voltage employed in said precipitation being such that the said unconsumed carbon is collected in a finely divided form.

3. In the art of producing lampblack, 95 that step in the art which consists in electrically precipitating carbon suspended in a gas in such a finely divided form that the precipitated particles can be removed without moving them with respect to each other and without a disruptive discharge, the voltage employed in said precipitation being from fifty thousand to seventy-five thousand 100 volts, the electric discharge used being of a non-disruptive character.

4. In the art of producing lampblack, 105 that step in the art which consists in electrically precipitating carbon particles suspended in a gas in such a finely divided form that the particles can be removed without removing them with respect to each other and without a disruptive discharge, 110 and dislodging the precipitated carbon without agitating them with respect to each other, the electric discharge used in said precipitation being of a non-disruptive character.

5. A method of producing lampblack by the incomplete combustion of a hydrocarbon in which the gaseous products resulting from the incomplete oxidation of a hydrocarbon and containing from two to three pounds of suspended unoxidized carbon particles for 1000 cubic feet are caused to impinge upon a cool surface until substantially one pound of said carbon particles per every 1000 cubic feet of the said gaseous products is collected and then electrically precipitating the remainder of said unoxidized carbon particles, the voltage employed in said electrical precipitation being such

that the carbon is collected in a finely divided form.

6. In the art of producing lampblack, that step in the art which consists in electrically precipitating unconsumed carbon suspended in a gas, the collecting surface being at zero potential, and the voltage employed being such that the carbon is collected in a finely divided form.

10 7. A method of producing lampblack which consists in electrically precipitating the unoxidized carbon particles suspended

in the gaseous products resulting from the incomplete oxidation of a hydrocarbon, said gaseous products being cooled to substantially 400° C. before the said electrical precipitation takes place, the voltage employed in said precipitation being such that the unoxidized carbon particles are collected in a loose and finely divided form. 15

In testimony whereof I hereunto affix my signature.

JULIAN M. GERARD.